

# UNITED STATES PATENT OFFICE.

GUSTAV CHAUDOIR, JR., OF VIENNA, AUSTRIA-HUNGARY.

## COPPER ALLOY.

No. 820,954.

Specification of Letters Patent.

Patented May 22, 1906.

Application filed February 3, 1904. Serial No. 191 911.

*To all whom it may concern:*

Be it known that I, GUSTAV CHAUDOIR, Jun., a subject of the King of Belgium, residing at Vienna, in the Province of Lower Austria and Empire of Austria-Hungary, have invented 5 certain new and useful Improvements in Copper Alloys, of which the following is a specification.

My invention relates to alloys of cadmium 10 with copper and the ordinary alloys of copper—viz., bronze and brass.

It is a well-known fact that the tensile strength of copper and its ductility decrease rapidly when the temperature of the metal is 15 raised. Tests carried out on a testing-machine, admitting of the metal being heated to any desired temperature, have shown that copper which at the temperature of 15° centigrade has a tensile strength of 38.1 kilo- 20 grams per square millimeter has only a tensile strength of 15.3 kilograms per square millimeter at a temperature of 500° centigrade.

Now my invention has for its object to effect an increase in the tensile strength and 25 ductility of copper and of its common alloys (bronze and brass) at high temperatures.

By conducting a series of experiments I have found that the purpose in view is advantageously attained by alloying copper, 30 bronze, and brass with cadmium in certain proportions.

I am aware that the specification of British Patent No. 10,197 of 1897 indicates alloys of copper which besides other metals contain 35 at most 0.5 per cent. of cadmium, the said

alloys being utilized in the manufacture of dynamo-brushes and their special composition having the effect of lessening the friction between the brushes and collectors or commutators. However, the alloys referred to 40 are on account of their too low percentage of cadmium quite unfit for the attainment of the purpose in view.

According to my invention from three-fourths to three and one-half per cent. of cadmium are added to the copper and to its common alloys, (bronze and brass.) By this addition the tensile strength of copper at the temperature of 500° centigrade is increased to 30.3 kilograms per square millimeter. The 50 increase of the ductility is especially conspicuous in the alloys richer in cadmium.

An alloy containing ninety-two parts of copper, four and one-half parts of tin, and three and one-half parts of cadmium has 55 shown especially good results.

What I claim, and desire to secure by Letters Patent of the United States, is—

A copper alloy containing from three-fourths to three and one-half parts of cadmium per from ninety-nine and one-fourth to ninety-two parts of copper. 60

In testimony whereof I have signed my name to this specification in the presence of two subscribing witnesses.

GUSTAV CHAUDOIR, JR.

Witnesses:

VICTOR KERPL,  
ALVESTO S. HOGUE.